

# United States Patent [19]

Berkes et al.

[11] B 3,923,512

[45] Dec. 2, 1975

[54] IMAGE RECORDING PROCESS

[75] Inventors: **John S. Berkes**, Webster; **William J. Hillegas**, Fairport; **Samuel W. Ing**, Webster, all of N.Y.

[73] Assignee: **Xerox Corporation**, Stamford, Conn.

[22] Filed: **Aug. 23, 1972**

[21] Appl. No.: **283,124**

[44] Published under the Trial Voluntary Protest Program on January 28, 1975 as document no. B 283,124.

## Related U.S. Application Data

[62] Division of Ser. No. 129,184, March 29, 1971, abandoned.

[52] U.S. Cl..... **96/27 R**; 96/90 PC; 96/88

[51] Int. Cl.<sup>2</sup> ..... **G03G 13/00**

[58] Field of Search..... 96/27 R, 1.5, 88, 90 PC

[56]

## References Cited

### OTHER PUBLICATIONS

C. A., 1934, 28, 4315.

C. A., 1923, 17, 928.

C. A., 1922, 16, 2244.

British Journal of Photography, 4/49, p. 188.

*Primary Examiner*—Charles L. Bowers, Jr.

*Assistant Examiner*—John L. Goodrow

*Attorney, Agent, or Firm*—James J. Ralabate; James P. O'Sullivan; Jerome L. Jeffers

[57]

## ABSTRACT

A method of imaging which comprises exposing an amorphous or crystalline chalcogenide layer to a pattern of light having wavelengths less than the band gap radiation of said chalcogenide, whereby the optical density of the layer is increased in the areas exposed to the light to form a visible image.

**13 Claims, No Drawings**

## IMAGE RECORDING PROCESS

This is a division of application Ser. No. 129,184 filed Mar. 29, 1971 now abandoned.

## BACKGROUND OF THE INVENTION

This application relates to a novel image recording process.

The instant invention is somewhat related to both xerography and silver halide photography, but has certain advantages and distinctions over both of these imaging systems.

In the art of xerography, a xerographic plate which contains a photoconductive insulating layer is imaged by first uniformly electrostatically charging the photoconductive surface. The plate is then exposed to a pattern of activating electromagnetic radiation such as light, which selectively dissipates the charge in the illuminated areas of the photoconductive insulator while leaving behind a latent electrostatic image in the non-illuminated areas. This latent image may then be developed to form a visible image by depositing a finely divided electroscopic marking particles on the surface of the photoconductive insulating layer. This concept was originally described by Carlson in U.S. Pat. No. 2,297,691 and is further amplified and described by many related patents in the field.

In silver halide photography, exposure of a silver halide emulsion layer to light, even for a short time, activates the silver halide particles so that they are much more easily reduced than before activation with the light exposure. This latent image which is formed by the exposure to light is then developed by washing the plate in a mild reducing agent, such as hydroquinone or pyrogallol, which has the ability to reduce the silver ions in those grains of silver halide upon which the light has fallen, while those grains which have not been struck with light are left unchanged. As a result of the developing process, the image appears upon the plate and is formed by a deposit of finely divided silver which is proportional in thickness to the intensity of light which fell upon each part of the plate. Any portion of the original object which was white will appear black upon the image, and because of this reversal of colors, the plate is called a negative. Before the negative can be brought out in the dark room, it is exposed to a solution of sodium thiosulfate which dissolves any unchanged silver halides, but has no affect upon the metallic silver of the image.

Both of the imaging processes defined above have particular application or utility in reproducing an image, as can be seen from the description of each technique. In order to produce a second or duplicate image in xerography, the entire xerographic process must be repeated a second time. In other words, as many duplicates as desired may be made by simply repeating all the process steps for the formation of each additional image. On the other hand, in forming a reproduction or photograph of an image by silver halide photography, the process for a given exposure is irreversible in that only one silver halide image may be formed from a given sheet of film. It can therefore be seen that for both xerography and silver halide photography, additional processing steps are required after image exposure. In order to form multiple or duplicate images in both techniques, either the entire process sequence must be repeated as in xerography; or as in silver halide

photography, a second or separate sheet of film must be used in order to reproduce a given image a second time.

In addition to the above, both xerography and silver photography have particular limitations with regard to their ultimate imaging resolution. For example, in xerography, the particle size of the toner will establish the resolution limit. In silver halide photography, the ultimate resolution of this system is directly related to the discrete particle size of the silver halide material.

It can be seen from the above that there exists a need for an imaging system in which images having high resolution can be formed by more simple and direct techniques.

There has now been discovered an imaging recording process by which visible images may be formed by single exposure to imaging light with no subsequent development of any type being required.

## OBJECT OF THE INVENTION

It is, therefore, an object of this invention to provide a novel imaging system which overcomes the above noted disadvantages.

It is another object of this invention to provide a novel imaging system by which a visible image is formed directly from a single exposure to imaging light.

It is a further object of this invention to provide an imaging system which does not require image development.

It is a further object of this invention to provide a novel imaging system which has recycling characteristics and which allows for images to be formed directly from a single exposure to imaging light.

It is another object of this invention to provide an imaging system having ultra-high resolution capability.

## SUMMARY OF THE INVENTION

The foregoing objects and others are accomplished in accordance with this invention by providing an amorphous or crystalline chalcogenide layer which undergoes a photochemical reaction when exposed to light of wavelengths less than the band gap radiation of the particular amorphous or crystalline material. The band gap radiation may also be described as the effective electronic energy gap. This wavelength or wavelength range is the point at which a given material exhibits the onset of carrier generation. It has been found that when these amorphous or crystalline layers are exposed to such radiation, a photochemical reaction occurs in the exposed areas which changes the reflectivity of the surface and increases the optical density of the film when viewed in transmission. Since the changes caused by the radiation occur in the region exposed to light, an image recording or photographic system results. Images formed by this technique may be stored indefinitely or may be viewed or reconstructed immediately.

The reconstruction of the image can be made with light whose wavelength is either shorter or longer than the band gap radiation used to form the image. Wavelengths which are longer than the band gap radiation of the particular material are preferred in that they provide superior image contrast. When desiring to use the film for an additional or added image, the original image may be removed by simply heating the imaging film which effectively erases the visible image.

60 The reconstruction of the image can be made with light whose wavelength is either shorter or longer than the band gap radiation used to form the image. Wavelengths which are longer than the band gap radiation of the particular material are preferred in that they provide superior image contrast. When desiring to use the film for an additional or added image, the original image may be removed by simply heating the imaging film which effectively erases the visible image.

## DETAILED DESCRIPTION OF THE INVENTION

The instant invention is directed to an imaging system which utilizes the photochemical reaction which occurs in both amorphous and crystalline forms of various chalcogenide systems when exposed to light in the wavelength region of less than the band gap radiation for the particular material. For purposes of this invention chalcogenides may comprise any materials made up of sulfides, selenides, tellurides or mixtures thereof. In addition, when in the vitreous form, these chalcogenide systems may vary widely from their stoichiometry. The exposure to light in the form of an image results in a change of the reflectivity of the surface of the material and increases the optical density of the film when viewed in transmission. For example, amorphous films of arsenic triselenide and arsenic trisulfide exhibit a change in surface reflectivity which is sometimes associated with a topographical smoothing of the surface in the radiation struck areas. The illuminated area when viewed in transmitted light exhibits an increase in optical density. Images formed by this method can be effectively erased by heating which renders the layer ready to be imaged a second time.

Although the theory of the above mechanism is not fully understood, it is believed that the change in optical density in the light struck areas is the result of phase separation in the region in which light is absorbed. For example, in arsenic triselenide, it is believed that very small particles of elemental arsenic are suspended in a matrix of amorphous selenium or arsenic-enriched selenium glass. The removal of the optical densified region by heating probably occurs by the process where all of the arsenic is taken back into solution by the selenium. This process will produce a homogeneous amorphous material identical to the film before it was illuminated, provided no arsenic has been lost. This effect has been observed for arsenic trisulfide.

In one embodiment, thin amorphous films of the above identified materials are formed in a thickness of several microns on any suitable support substrate. The support may comprise any suitable conductive or insulating material. Typical conductive materials include brass, aluminum, steel or the like. The amorphous films may be contained on a rigid or flexible supports and in any suitable form such as a sheet, web, cylinder, or the like. Inasmuch as there is no necessary chemical reaction between the amorphous film and substrate, or any necessary electrical requirements, it is preferred that the substrate comprise a dielectric material such as glass, aluminum oxide, a ceramic, plastic, or any other suitable dielectric. If the image is to be used in transmission it is also preferred that the substrate be transparent. When used in the amorphous form, devices employing amorphous layers may comprise any suitable chalcogenide system. Typical compositions include arsenic triselenide, cadmium selenide, gallium selenide, arsenic trisulfide, arsenic telluride, cadmium sulfide, antimony sulfide, antimony selenide, antimony telluride, bismuth sulfide, bismuth selenide, bismuth telluride, germanium sulfide, germanium selenide, germanium telluride, and mixtures thereof such as ternary, quaternary and more complex systems defined by all combinations of these materials. For example, these might include ternaries containing arsenic-bismuth-selenide or arsenic-germanium-telluride, etc.

The band gap radiation for arsenic trisulfide is about 5300 Angstrom Units, while the band gap radiation for

arsenic triselenide is about 7100 Angstrom Units. For the various chalcogenide systems of the instant invention, the band gap radiation varies from about 5000 to 10,000 Angstrom Units. Since the photochemical reaction is essentially temperature independent, images can be formed at all temperatures below the liquidus or fusion temperature and images have been formed at temperatures as low as 120°K. Similarly, erasure of the image can be simply accomplished by heating the film to a temperature above the temperature at which the image is formed. The erasure temperature need not necessarily exceed the glass transition or liquidus temperature.

The thickness of the amorphous film is not particularly critical but thicknesses in the range of about 1 to 10 microns have been found to yield particularly satisfactory results. When viewed in transmission with visible light, however, the non-imaged areas must be transparent to the reading light and consequently thinner samples may be necessary for materials which have a band gap in the red.

The amorphous layers of the instant invention may be prepared by any suitable technique. A preferred technique includes vacuum evaporation wherein the composition forming the amorphous layer is evaporated onto a suitable base material or support. In general, the vacuum conditions may vary from about  $10^{-5}$  to  $10^{-8}$  Torr. In one embodiment, a master alloy comprising the appropriate ratio of the two or more materials of the amorphous layer is first made. The master alloy is then vacuum evaporated onto a supporting substrate maintained at relatively low temperature in the range of about 20° to 80°C. In another embodiment called co-evaporation, separate elemental sources of the two components which make up the final layer are placed in separate heated crucibles and maintained under vacuum conditions with a source temperature of each alloy constituent being controlled so as to yield the appropriate percentage or proportion of the alloy desired.

Another typical method of making amorphous layers of the instant invention includes flash evaporation under vacuum conditions which are similar to those defined in co-evaporation. In this technique, a powdered alloy such as arsenic triselenide is selectively dropped into a heated crucible maintained at a temperature in the range of about 300° to 600°C. The vapors formed from the heated mixture are evaporated upwards onto a substrate supported above the crucible.

In all of the above evaporation techniques, the substrate onto which the photconductive material is evaporated is usually maintained at a temperature of about 20° to 80°C. If desired, a water cooled platen or other suitable cooling means may be used in order to maintain a constant substrate temperature. In general, an amorphous arsenic selenide layer approximately 5 microns thick is obtained when vacuum evaporation is carried out for about 30 minutes at a vacuum of about  $10^{-8}$  Torr and a crucible temperature of about 400°C. In general, crucibles which are used for evaporation of amorphous layers may be of any inert material such as quartz, molybdenum, stainless steel, or stainless steel coated with a layer of silicon monoxide.

In imaging the amorphous layers of the instant invention, the layer must be exposed to light in the wavelength region which is less than the band gap radiation. This range is required in order for the photochemical reaction to occur and cause a change in reflectivity of

the surface in the light struck areas. In general, the greater the intensity of the exposing light, the shorter time duration required for exposure. For example, when using ordinary tungsten light from an optical microscope, the light intensity is rather low and hence a rather long time period, sometimes several hours or more, is required. On the other hand when using a high intensity light source such as a laser, the imaging may be carried out in a matter of seconds or minutes. It therefore follows that as the intensity of the imaging light becomes greater, the density of the image increases.

Amorphous films of the instant invention can be viewed or reconstructed immediately with no further development step being required after the initial exposure. The reconstruction of the image can be made with light whose wavelength is preferably longer than the band gap radiation. If desired, the image can be erased by heating the member containing the amorphous film. After erasure of the image the member is ready for subsequent imaging. Because the entire amorphous layer is active or sensitive to light, the resolution of images formed by the technique of the instant invention should approach the precipitate dimensions of the material. This high resolution capability has utility in microrecording systems such as in holographic and memory devices. Resolutions of 70 line pairs per millimeter have been demonstrated. The theoretical resolution limit would be determined by the perfection of the evaporated film and should be greater than about 200 line pairs per millimeter. In general, the stability of images formed by this technique when kept at room or ambient conditions will not normally deteriorate in any known time period. For example, images have been made and stored for 18 months with no degradation in image quality being observed.

When using samples of crystalline chalcogenides, the samples may be prepared by any conventional techniques which are used for forming crystalline materials. For example, crystals of arsenic triselenide may be formed by first taking a master alloy having the appropriate ratio of arsenic and selenium (i.e.  $As_2Se_3$ ) and placing the master alloy in a sealed quartz ampul. The ampul containing the alloy is placed in an oven maintained at 336°C. for 7 days. At the end of this time the ampul is cooled, broken open, and a number of arsenic triselenide crystals which have been formed by vapor transport, are removed from the ampul. Crystals of arsenic sulfide are formed by the above method by heating at a temperature of 250°C. In addition, 1.0 percent thallium is added to the alloy in order to insure crystal formation.

#### DESCRIPTION OF THE PREFERRED EMBODIMENTS

The following examples further specifically define the present invention with respect to a method of making and imaging amorphous films of chalcogenide systems.

#### EXAMPLE 1

A master alloy of arsenic triselenide is made by weighing out 40 atomic percent of arsenic and 60 atomic percent of selenium. Both the arsenic and selenium are substantially pure materials having a purity of about 99.999 percent. The arsenic and selenium are then placed into a clean, fused silica ampul. The ampul is then evacuated to a pressure of about  $10^{-8}$  Torr and

sealed. The sealed ampul is then placed into a furnace which is heated to a temperature of about 600°C. in a period of about 3 hours. To aid in the reaction of the arsenic and selenium and to assure alloy uniformity, the furnace is rocked for about a 12 hour period at 600°C after which the ampul is removed from the furnace and quenched in water at room temperature. The alloy is then removed from the ampul, crushed, and is then ready for use as a master alloy of arsenic triselenide for vacuum evaporation.

#### EXAMPLE 2

A master alloy of arsenic trisulfide is formed by the method of Example 1 using a ratio of 40 atomic percent arsenic and 60 atomic percent sulfur.

#### EXAMPLE 3

A series of three amorphous arsenic triselenide films 20 1 to 2 microns thick contained on a pyrex glass substrate are made by the following technique. A sample of the master alloy of arsenic triselenide formed by Example 1 is placed in a stainless steel boat which is inserted into a vacuum chamber. A pyrex glass substrate is suspended about 12 inches above the boat and the chamber evacuated to a vacuum of about  $10^{-5}$  Torr. The stainless steel boat containing the arsenic triselenide is then heated to a temperature of about 400°C. for about 10 minutes. The substrate is maintained at a temperature of about 20° to 25°C. during the evaporation process. At the end of the evaporation cycle, the vacuum chamber is cooled to room temperature, the vacuum broken, and the pyrex substrate containing an amorphous film about 1 to 2 microns thick of arsenic triselenide is removed from the chamber. This process is repeated two additional times to form a total of three arsenic triselenide plates contained on pyrex glass substrates. A fourth plate is made as above using an aluminum oxide wafer as the substrate.

#### EXAMPLE 4

The method of Example 3 is used to form a 5 micron thick layer of arsenic trisulfide contained on an aluminum oxide wafer. The stainless steel crucible is heated to a temperature of about 350°C.

#### EXAMPLE 5

A plate formed by Example 3 which contains an amorphous film or amorphous arsenic triselenide contained on the pyrex glass substrate is imaged by the following technique. A test pattern is formed by projection onto the arsenic triselenide surface by using a light source containing a tungsten lamp having at 20 watt output. The light is focused onto the amorphous surface and a test pattern projected at 1:1 magnification onto the arsenic triselenide film with f/2.8 optics. The projection method is similar to that used for a standard 50 slide projector. This image technique is carried out for an exposure 1 hour at under atmospheric conditions at a temperature of about 23°C. This resultant image is stable and exhibited no noticeable deterioration after 18 months of storage under room ambient conditions in a light tight container. The image quality of the test pattern was sharp and has a resolution of about 70 line pairs per millimeter when observed through a microscope.

## EXAMPLE 6

A second sample formed by Example 3 containing an amorphous arsenic triselenide film contained on pyrex glass is imaged by contact printing using the following technique. A light image is formed by focusing a microscope light using a tungsten light source from a Leitz Ortholux Microscope using a 5x objective. The exposure is for a time period of 15 minutes under atmospheric conditions at a temperature of 23°C.

The image of the letter "x" from the contact image source is recorded on the film. When viewed in transmitted visible light this "photograph" appears as a black letter on a lighter background.

## EXAMPLE 7

Using a 5 micron film of arsenic trisulfide contained on an aluminum oxide wafer substrate (Example 4), a contact print was formed by the following technique. A light image was formed by focusing microscope light from a tungsten filament using a Leitz Microscope with a 5x objective. The exposure time is for a period of 2 hours under atmospheric conditions at a temperature of 23°C.

The image is similar to that described in Example 6 above.

## EXAMPLE 8

A sample containing an amorphous layer of arsenic triselenide contained on the pyrex glass substrate (Example 3) is imaged by a laser beam using the following technique. The laser beam contains a light source of 4579 Angstrom Units and a light intensity of  $10^{16}$  (photons/cm<sup>2</sup> sec.) using an exposure time of 3 seconds at a temperature of 25°C under atmospheric conditions. A clearly visible image consisting of a dark spot the size of the laser beam (about 2mm in diameter) is visible when the filter is viewed in transmitted visible light.

## EXAMPLE 9

A sample containing a 1 micron layer of arsenic triselenide contained on an aluminum oxide substrate wafer (Example 3) are imaged by a laser beam as follows. The laser beam has a wavelength of 6328 Angstrom Units and a light intensity of  $10^{16}$  (photons/cm<sup>2</sup> seconds) at a temperature of 120°K under a vacuum of  $10^{-4}$  centimeters of mercury. An exposure time of 20 seconds results in a relative transparency of 0.75 compared to the virgin material.

In addition to the above imaging, the image can be erased by heating the sample to 250°K and subsequent cooling to 120°K. The same results can be obtained by carrying out the initial exposure at 298°K. Erasure can be achieved by heating to 400°K and subsequently cooling back to 298°K. The reaction responsible to the reversibility is at least as fast as the heating rate (about 1°K/min.) which is used in the experiment.

## EXAMPLE 10

An arsenic trisulfide crystal having a needlelike shape about 3 millimeters long and a cross-section of about 0.2 millimeters is illuminated by focusing the microscope light on a portion of the crystal by the illumination technique described in Example 7. The crystal is exposed for about 12 hours which results in the formation of a dark spot about 0.3 millimeters long when the crystal is viewed in reflected light. This experiment is repeated using an arsenic triselenide crystal. The results

are similar to those observed for the arsenic trisulfide crystal.

Although specific components and proportions have been stated in the above description of the preferred embodiments of this invention, other suitable materials and procedures such as those listed above may be used with similar results. In addition, other materials and changes may be utilized which synergize, enhance, or otherwise modify the above techniques.

10 Other modifications and ramifications of the present invention would appear to those skilled in the art upon reading the disclosure. These are also intended to be within the scope of this invention.

## What is claimed is:

15 1. A method of imaging which comprises exposing an amorphous layer of arsenic trisulfide to a pattern of light having wavelengths less than the bandgap radiation of said arsenic trisulfide, whereby the optical density of the amorphous layer is increased in the areas exposed to the light to form a visible image and heating the imaged layer to a temperature above that at which the image was formed to erase the image.

20 2. A method of imaging which comprises exposing a crystalline layer of arsenic triselenide to a pattern of light having wavelengths less than the bandgap radiation of said arsenic triselenide, whereby the density of the crystalline layer is increased in the areas exposed to the light to form a visible image and heating the imaged layer to a temperature above that at which the image was formed to erase the image.

25 3. The method of claim 1 wherein the light has wavelengths of less than 5300 Angstrom units.

4. The method of claim 1 in which the amorphous layer is contained on the dielectric substrate.

5. The method of claim 1 wherein the amorphous layer is contained on a dielectric substrate.

6. The method of claim 2 wherein the light has wavelengths of less than 7100 Angstrom units.

30 7. The method of claim 2 wherein the image is erased by heating the amorphous layer to a temperature in the range of about 100° to about 120°C. greater than the exposure temperature.

8. The method of claim 1 in which the image is erased by heating the amorphous layer to a temperature in the range of about 100 to 120°C greater than the exposure temperature.

9. The method of claim 2 wherein the crystalline layer is contained on a dielectric substrate.

50 10. A method of imaging which comprises exposing a layer of an amorphous or crystalline chalcogenide material selected from the group of sulfides, selenides or tellurides of arsenic, antimony, bismuth, gallium or germanium to a pattern of light having wavelengths of less than the bandgap radiation of said chalcogenide, said light having sufficient intensity to cause a photochemical reaction in the light struck areas, whereby the optical density of the layer is increased in the areas exposed to light resulting in the formation of a visible image and heating the imaged layer to a temperature above that at which the image was formed to erase the image.

55 11. The method of claim 9 wherein the chalcogenide is selected from the group of arsenic triselenide, cadmium selenide, gallium selenide, arsenic trisulfide, arsenic telluride, cadmium sulfide, antimony sulfide, antimony selenide, antimony telluride, bismuth sulfide, bismuth selenide, bismuth telluride, germanium sulfide, germanium selenide, germanium telluride and mixtures thereof.

12. The method of claim 9 in which the layer is contained on a dielectric substrate.

13. The method of claim 9 wherein the image is erased by heating the layer to a temperature in the

range of about 100° to 120°C. greater than the exposure temperature.

\* \* \* \* \*